

Aug. 26, 1941.

C. A. MEDSKER

2,253,526

METHOD OF MAKING COMPOSITE METAL SLABS

Filed June 22, 1939

2 Sheets-Sheet 1



Aug. 26, 1941.

C. A. MEDSKER

2,253,526

METHOD OF MAKING COMPOSITE METAL SLABS

Filed June 22, 1939

2 Sheets-Sheet 2



Fig. 3



Fig. 5



Fig. 6



Fig. 7

INVENTOR.  
CHARLES A. MEDSKER

BY

Horace B. Fay  
ATTORNEY.

## UNITED STATES PATENT OFFICE

2,253,526

## METHOD OF MAKING COMPOSITE METAL SLABS

Charles A. Medsker, Cleveland Heights, Ohio,  
assignor to William L. Ulmer, Cleveland, Ohio

Application June 22, 1939, Serial No. 280,593

8 Claims. (Cl. 22—204)

This invention relates, as indicated, to a method of making composite metal slabs.

A primary object of the invention is to provide a method whereby composite metal slabs characterized by an extremely strong bond between the component metals thereof, may be easily and quickly made in a continuous or intermittent manner.

To the accomplishment of the foregoing and related ends, said invention, then, consists of the steps hereinafter fully described and particularly pointed out in the claims; the annexed drawings and the following description setting forth in detail one mode of carrying out the invention, such disclosed mode illustrating, however, but one of various ways in which the principle of the invention may be used.

In said annexed drawings—

Fig. 1 is a side elevational view of apparatus embodying the invention;

Fig. 2 is a transverse cross-sectional view of the apparatus, taken on the line 2—2 of Fig. 1;

Fig. 3 is a plan view of the apparatus;

Fig. 4 is a perspective view, on an enlarged scale, of one of the portable slab molds;

Fig. 5 is a transverse cross-sectional view of the mold, taken on the line 5—5 of Fig. 4;

Fig. 6 is a perspective view of a modified form of slab mold; and

Fig. 7 is a transverse cross-sectional view, taken on the line 7—7 of Fig. 6.

Referring more particularly to the drawings, the apparatus is seen to comprise a supporting framework 1 consisting of structural members suitably secured together, and having mounted thereon a pair of transversely spaced longitudinally extending rails 2, which serve a purpose to be presently described.

Extending transversely of the framework 1, adjacent the ends thereof are shafts 3, carrying sprocket wheels 4, in engagement with which is an endless conveyor chain 5, the chain being disposed intermediate the sides of the framework, and the upper run of the chain being disposed at a level somewhat above that of the rails 2. The shaft 3 at the right end of the framework drives the chain 5, and is in turn driven by a motor 6 through the intermediary of a speed reduction unit 7.

Supported on the framework 1 is a second pair of transversely spaced longitudinally extending rails 8, these rails being disposed directly below the rails 2 and being at a level considerably below the lower run of the conveyor chain 5.

Surrounding the upper forward portion of the

framework and conveyor chain is a preheating furnace which is supported at its ends by legs 10. A combustible gas is adapted to be supplied to the furnace as by means of burner pipes 11, which, in turn, are supplied by a manifold conduit 12, each of the pipes 11 being provided with a hand-controlled valve 13 for regulating the supply of gas thereto. A portion of the gas supply from the manifold 12 is by-passed through a conduit 14 and a fluxing device 15, which may be similar to the devices described in my co-pending application Serial No. 261,559, and as a result of which a flux is entrained in the gas. Such flux is desirably a vapor phase flux of the character described in the co-pending applications of Bialosky and Sobel, Serial Nos. 220,560 and 228,398.

The gas, having a flux entrained therein, upon leaving the fluxing device 15 passes through a conduit 16 which terminates in a horizontally disposed burner 17, overlying and extending transversely of the framework 1, at a point spaced from the exit end of the furnace 9. The burner 17 is provided with a series of downwardly and forwardly inclined spaced jets 18 through which the gas having the flux entrained therein emerges, and at which such gas is burned.

Another portion of the gas supply from the manifold 12 is passed directly through a conduit 18, which terminates in a horizontally disposed burner 19, overlying and extending transversely of the framework 1 at a point spaced forwardly of the burner 17. The burner 19 is provided with a series of downwardly and rearwardly inclined spaced jets 20, through which the gas emerges and at which it is burned.

Disposed at the side of the framework 1 of the apparatus, at a point opposite the burners 17 and 19, is an electric melting furnace 21 having trunnions 22, journaled on pedestals 23, whereby the furnace may be tilted to discharge the molten contents thereof through the spout 24 and into one of the molds to be now described.

Each mold comprises a shallow rectangular open top box 25, formed of a suitable refractory material, and having a rectangular opening 26 in the central portion of the bottom thereof. Each mold has secured thereto a pair of spaced shafts 27, each shaft being provided with flanged wheels 28, which rest on the rails 2 for facilitating movement of the molds along the framework 1. Each mold is provided with a pair of upwardly extending lugs 29 and a pair of down-

wardly extending lugs 30, which serve a purpose to be presently described.

The apparatus further includes a hydraulically operated loading platform or station 31, positioned in front of the furnace 9, and an unloading platform or station 32, having an opening 33 thereon, corresponding in size with the mold openings 26, the platform 32 being supported by pistons 34, which operate in cylinders 35, the pistons being actuated by means of a fluid admissible into and withdrawable from the cylinders through a conduit 36.

For the purpose of ejecting the slabs from the molds, a hydraulically operated ram 37 is provided, the fluid for the operation of which is supplied by means of a conduit 38.

For the purpose of cooling the composite slabs, a conduit 39 is provided, which overlies the framework at a point intermediate the furnace 21 and the unloading platform 32, and through which water is sprayed onto the slabs.

The operation may now be described as follows:

With the mold 25 positioned on the platform 31, as shown in Fig. 1, a slab of steel or other metal is placed in the mold, such slab being designated by the reference character S in Fig. 5, the upper surface of such slab having been previously prepared, as by suitable machining and cleaning operations. The platform is then elevated until the mold is on a level with the upper run of the conveyor chain 5, after which the mold is pushed into the preheating furnace 9, with the wheels 28 thereof resting on the rails 2. The lugs 30 of the mold are engaged by the conveyor chain 5, and in this way the mold is caused to slowly traverse the furnace, the slab S being heated up to a desired temperature.

The mold with the hot slab S therein, is then moved to a position opposite the furnace 21, and, while burning gas, having flux entrained therein, is directed against the upper surface of the slab S, the furnace 21 is tilted so as to cause the contents thereof, or at least a portion of such contents to flow into the mold, and onto the slab S. The metal, thus poured onto the slab, may be copper or some other material different from the metal of the slab S, and, due to the action of the vaporizing flux, such metal becomes firmly bonded to the slab S. The burning gases, issuing from the burners 17 and 19, are of value in preserving the metal poured onto the slab S in molten condition for a sufficient length of time to permit it to spread evenly over the slab, forming a layer C (see Fig. 5) of such metal.

The mold with the composite slab therein then proceeds to a point below the conduit 39, where the slab is cooled by the water issuing from said conduit.

The mold then passes onto the unloading platform 32, and while the mold is thus positioned on the platform, the platform is lowered, while the ram 37 remains stationary. As the mold is thus lowered, the slab engages the ram, which projects upwardly through the opening 26 in the mold, with the result that the slab is ejected from the mold, and is exposed for removal to any desired point for further operations thereon, such as rolling.

The platform descends to the level of the rails 8, and the ram 37 is likewise lowered. The empty mold is then pushed onto the rails 8, where the lugs 29 thereof are engaged by the lower rim of the conveyor chain 5, the mold being in this way returned to the loading platform 31.

As will be apparent from Fig. 1, the operations

may be continuous or intermittent and in order to increase the productive capacity of the apparatus, a plurality of molds are provided.

The furnace 21 is preferably of a size suitable for melting sufficient metal to fill a large number of molds, and a neutral or reducing atmosphere is desirably maintained within this furnace.

The process thus includes the steps of preheating the backing metal slab, cladding or coating the preheated slab, and cooling the composite slab. If desired, the slab S, after being coated on one side with a cladding metal, may be inverted in the mold, and the other side clad or coated with a cladding metal of the same kind, or a different cladding metal.

Instead of using a mold, such as shown in Figs. 4 and 5, an adjustable mold, such as shown in Figs. 6 and 7, may be employed. Such a mold comprises a steel or platform 50 having mounted thereon side walls 51 and end walls 52, which are lined with refractory bricks 53. In order to vary the size of the mold, the walls 51 may be adjusted, and for this purpose each of these walls is provided with a plurality of bolts 54 having heads 55 which are movable in T-slots 56 in the platform 50. The walls 51 are maintained in adjusted position by means of nuts 57, which are secured to the bolts 54 and are drawn down into engagement with the walls. By substituting shorter or longer walls for the walls 51, the end walls 52 may also be adjusted to further change the size of the mold, additional T-slots 56, bolts 54 and nuts 57 being provided for this purpose.

The temperature to which the slab S should be preheated will vary both with the nature of the cladding metal and with the alloying affinity of the cladding metal with the metal of the slab. While high temperatures are at all times more desirable from the viewpoint of ease of surface alloying (and therefore of adhesion), the danger of surface oxidation of the slab also increases rapidly with high temperatures. The exact preheating temperature must therefore be a balance between these factors. Where it is possible to super-heat the cladding metal, the temperature of preheating of the base metal or slab can be correspondingly lowered, since the cladding metal, in such case, will supply the necessary heat to the bonding surface.

Certain metals and alloys tend to become alloyed with iron or steel more readily than others, and since this surface alloying is the criterion of bonding, the slab need not be heated to as high a temperature where such readily alloyable cladding metals and alloys are employed as would otherwise be the case. An example of this is the copper-zinc brass series. On the other hand, metals such as the silicon bronzes do not readily form surface alloys with iron or steel, and in such case, it is necessary to have as high a temperature at the bonding surface as can possibly be secured. This may be accomplished in two ways, i. e. either the slab itself may be heated to a relatively high temperature, with the cladding metal at a temperature only slightly above its melting point, or the slab can be heated to a relatively low temperature and the cladding metal heated to as high a temperature as is possible in the electric furnace, the only limitations in the heating of the cladding metal in such case, being the character of refractory used in the furnace and the volatilizability of the constituents of the cladding metal or alloy.

Where a temperature in excess of 800° F. is required for the preheating of the slab, it is desir-

able that flux of the character described be applied to the slab in the preheating furnace in which event the fluxer 15 is so placed that the gas will pass therethrough before entering the burner pipes 14. Moreover, instead of using a preheating furnace of the direct-fired type, as illustrated, a muffle type furnace may be employed in which a neutral or reducing atmosphere may be maintained, in which event, the flux may be entrained in the gases used for producing such an atmosphere, sufficient oxygen being introduced however to insure conversion of the organic borate in the flux to boric oxide.

The cladding metal may, under some circumstances, be poured onto the slab within the preheating furnace, which, in such case, is so constructed as to provide an inlet for the molten metal. Where the cladding metal is poured onto the slab exteriorly of the preheating furnace, as illustrated in the drawings, it is desirable and perhaps essential that the slab be fluxed at the point of pouring, irrespective of the fact that it has been fluxed while in the preheating furnace.

For cladding with metals containing volatile constituents, such as zinc-copper alloys, melting by an electric furnace is impractical, since the zinc will become volatilized and burned out. For cladding, with such metals, it is preferred to substitute for the electric furnace melting devices of lower temperature nature, such as gas-fired crucible furnaces, etc.

Other forms may be employed embodying the features of my invention instead of the one herein explained, change being made as regards the means and the steps herein disclosed, provided the elements stated by any of the following claims or the equivalent of such stated elements be employed, whether produced by my preferred method or by others embodying steps equivalent to those stated in the following claims.

I therefore particularly point out and distinctly claim as my invention:

1. A method of making a composite metal slab which consists in preheating a slab of steel to a desired temperature, pouring a molten metal predominant in copper onto said preheated slab of steel, and directing a combustible gas containing a vaporized flux onto the surface of said steel slab during said pouring operation.

2. A method of making a composite metal slab which consists in preheating a metal slab, directing a combustible gas containing a vaporized flux onto the upper surface of said slab, and during

the course of such treatment with flux, pouring a second metal, in molten condition, onto said slab.

3. A method, as in claim 2, in which the composite slab is cooled with water to hasten the solidification of the applied metal.

4. A method of making a composite metal slab which consists in preheating a slab of steel to a desired temperature by means of a combustible gas containing a vaporized flux and then pouring a molten metal predominant in copper onto said preheated slab of steel.

5. A method of making a composite metal slab which consists in directing a combustible gas containing a vaporized flux onto the upper surface of said slab, and then pouring a second metal, in molten condition, onto said slab.

6. In a method of cladding metals, the steps which consist in providing a backing metal and a metal to be applied thereto, thoroughly cleaning substantially the entire surface of said backing metal of all impurities which would interfere with the creation of a sound bond between the backing and applied metal by directing a combustible gas flame having a vaporized flux entrained therein against said surface, and flowing said metal to be applied onto said backing metal in such a manner as to cause said applied metal to cover substantially all of said cleaned surface.

7. The process of cladding metals which comprises providing a base metal and a metal to be applied thereto, maintaining said base metal in an unfused state, subjecting substantially the entire surface of said base metal to the action of a combustible gas flame having a vaporized flux entrained therein, and, while said base metal is under the influence of said flame and flux, applying said metal to be applied onto said base in such a manner as to cover substantially the entire surface of said base metal.

8. The process of cladding metals which comprises providing a base metal and a metal to be applied thereto, maintaining said base metal in an unfused state, subjecting substantially the entire surface of said base metal to the action of a combustible gas flame having a vaporized flux entrained therein, and, while said base metal is under the influence of said flame and flux, flowing said metal to be applied onto said base in such a manner as to cover substantially the entire surface of said base metal.

CHARLES A. MEDSKER.